



US008430768B2

(12) **United States Patent**  
**Komatsu et al.**

(10) **Patent No.:** **US 8,430,768 B2**  
(45) **Date of Patent:** **Apr. 30, 2013**

(54) **COLOR GOLF BALL**

(75) Inventors: **Atsushi Komatsu**, Chichibu (JP);  
**Hirosi Nasu**, Shinagawa-ku (JP)

(73) Assignee: **Bridgestone Sports Co., Ltd.**, Tokyo  
(JP)

(\*) Notice: Subject to any disclaimer, the term of this  
patent is extended or adjusted under 35  
U.S.C. 154(b) by 254 days.

(21) Appl. No.: **12/854,523**

(22) Filed: **Aug. 11, 2010**

(65) **Prior Publication Data**

US 2010/0323821 A1 Dec. 23, 2010

**Related U.S. Application Data**

(63) Continuation-in-part of application No. 12/818,289,  
filed on Jun. 18, 2010, which is a continuation-in-part  
of application No. 12/167,423, filed on Jul. 3, 2008,  
now Pat. No. 7,780,550.

(51) **Int. Cl.**  
**A63B 37/06** (2006.01)  
**A63B 37/04** (2006.01)

(52) **U.S. Cl.**  
USPC ..... **473/377; 473/378; 473/371; 473/376**

(58) **Field of Classification Search** ..... None  
See application file for complete search history.

(56) **References Cited**

**U.S. PATENT DOCUMENTS**

6,022,279 A \* 2/2000 Yamagishi et al. ..... 473/353  
6,435,984 B1 \* 8/2002 Ohama ..... 473/377  
6,558,277 B1 \* 5/2003 Ohira et al. ..... 473/378  
6,561,923 B1 \* 5/2003 Ohama et al. ..... 473/353  
6,676,543 B2 \* 1/2004 Endo ..... 473/378

6,716,116 B1 \* 4/2004 Yokota ..... 473/378  
7,160,210 B2 \* 1/2007 Melanson et al. ..... 473/378  
7,291,076 B2 11/2007 Watanabe

(Continued)

**FOREIGN PATENT DOCUMENTS**

|    |            |         |
|----|------------|---------|
| GB | 2121294 A  | 12/1983 |
| JP | 58218977 A | 12/1983 |

(Continued)

*Primary Examiner* — Alvin Hunter

*Assistant Examiner* — John E Simms, Jr.

(74) *Attorney, Agent, or Firm* — Sughrue Mion, PLLC

**ABSTRACT**

The invention provides a colored golf ball comprising a core, a cover having a plurality of dimples formed on its surface, wherein the golf ball is two-piece structure consisting of a core and a cover, and the surface of the ball is coated with a coating comprising a pearlescent pigment. The ball satisfies the following conditions:

- (i) a color difference  $\Delta E^*$  between the core and the ball of at least 30;
- (ii) the core has a transparency which is up to 10% in terms of total transmittance and up to 1.0% in terms of parallel transmittance;
- (iii) the core has a lightness  $L^*$  value, expressed in the  $L^*a^*b^*$  color system based on JIS Z8729, of at least 82;
- (iv) the ball has a lightness  $L^*$  value of at least 50;
- (v) the lightness  $L^*$  value of the ball  $\leq$  the lightness  $L^*$  value of the core;
- (vi) the cover has a thickness of from 0.1 to 2.1 mm;
- (vii) the cover has a transparency which is at least 50% in terms of total transmittance and at least 1.0% in terms of parallel transmittance; and
- (viii) the cover has a haze (H), mentioned in JIS K7105 (1981), of up to 98.

The two-piece colored golf ball of the invention is a fluorescent ball which nonetheless retains a sense of transparency and has a high-quality feel, in addition to which it has a good weather resistance and is capable of preventing a change in color.

**8 Claims, 4 Drawing Sheets**



**US 8,430,768 B2**

Page 2

---

U.S. PATENT DOCUMENTS

|                  |        |                 |         |    |               |         |
|------------------|--------|-----------------|---------|----|---------------|---------|
| 2003/0153402 A1* | 8/2003 | Simonds et al.  | 473/351 | JP | 2000-24139 A  | 1/2000  |
| 2007/0015603 A1* | 1/2007 | Watanabe et al. | 473/371 | JP | 2000-254250 A | 9/2000  |
| 2007/0135234 A1* | 6/2007 | Nagasaki et al. | 473/353 | JP | 2004-33594 A  | 2/2004  |
| 2009/0109379 A1* | 4/2009 | Fukagawa et al. | 349/96  | JP | 2004081350 A  | 3/2004  |
|                  |        |                 |         | JP | 3862332 B2    | 10/2006 |
|                  |        |                 |         | JP | 2007-21204 A  | 2/2007  |
|                  |        |                 |         | JP | 2007-21205 A  | 2/2007  |
|                  |        |                 |         | JP | 2007-144097 A | 6/2007  |

FOREIGN PATENT DOCUMENTS

|    |             |        |
|----|-------------|--------|
| JP | 6088567 A   | 5/1985 |
| JP | 10-155937 A | 6/1998 |

\* cited by examiner

**FIG.1****FIG.2**

**FIG.3**



**FIG.4**



**FIG.5**



**FIG.6**



**FIG.7**



**FIG.8**



# 1

## COLOR GOLF BALL

### CROSS-REFERENCE TO RELATED APPLICATION

This application is a continuation-in-part of copending application Ser. No. 12/818,289 filed on Jun. 18, 2010, which is a continuation-in-part of copending application Ser. No. 12/167,423 filed on Jul. 3, 2008, the entire contents of which are hereby incorporated by reference.

### BACKGROUND OF THE INVENTION

The present invention relates to a colored golf ball having a fluorescent color. More specifically, the invention relates to a fluorescent colored golf ball which is endowed with a coloring that conveys a sense of quality, performance attributes, and an excellent color change resistance.

Recently, color golf balls such as yellow, pink and orange have begun to be used, alternative to a white golf ball used in the conventional art. The reason why such color balls are used is that they are endowed with the psychological impression from the visibility and the color tone of the ball.

In addition, while golf balls having high performances exist, it is fact that many golfers still seek a two-piece golf ball because the two-piece golf ball is comparatively inexpensive owing to use rubbers in a major part of the material. Furthermore, in order to obtain an inexpensive two-piece golf ball, the cover is made thinner as one of the way for the inexpensive two-piece golf ball to be manufactured.

However, such two-piece golf ball satisfying "inexpensiveness" and "a color ball" lacks a high-quality feel and a resistance to color change. Also, the technique of the two-piece color ball of thinner cover was still insufficient.

Golf balls which have hitherto been disclosed include the following prior art.

JP-A 2007-21204, which describes a golf ball having a clear cover over a core that is coated with a bright pigment-containing coating, strives to achieve a metallic texture and markings that appear three-dimensional. The intention is not to provide a fluorescent colored ball.

JP-A 2007-21205 describes a golf ball in which the color difference  $\Delta E$  between an inside layer and the ball is set to a small value of 30 or less. However, this ball has a subdued appearance that lacks visual impact. Moreover, the object here is to include a pearlescent pigment in the cover so as to give the cover a pastel tone; it is not the object of this prior-art disclosure to use a fluorescent pigment or dye so as to achieve bright coloring having a high-quality feel.

In the golf ball disclosed in U.S. Published patent application Ser. No. 11/882,216, a large amount of fluorescent pigment is added to the cover, resulting in a less than adequate transparency and an excessively strong color tone which deprives the ball of a high-quality feel. Also, the addition of a large amount of fluorescent pigment gives the ball a poor resistance to color change.

The golf balls described in JP-A 2007-144097 and U.S. Published patent application Ser. No. 11/299,947 lack specificity concerning the cover transparency, in addition to which no mention whatsoever is made of a high-quality feel.

JP-A 10-155937, and JP-A 2000-254250 mention balls which exhibit pastel tones. However, these golf balls are very deeply colored and visually disconcerting. Moreover, they lack a high-quality feel and have a poor resistance to color change.

JP-A 2000-24139 discloses a colored ball of excellent visibility which has a bright, highly intense color tone. However,

# 2

because the cover contains a large amount of fluorescent pigment, it is not sufficiently transparent and has an excessively strong color, resulting in a ball that lacks a high-quality feel.

JP-A 2004-33594 describes a golf ball of blue, pink or yellow color which is specified in terms of the  $L^*a^*b^*$  color system so as to enhance visibility. However, such golf balls do not excel in terms of a high-quality feel, performance and resistance to color change.

JP-A 2009-45347 describes a golf ball having a high chroma and a high-quality feel by painting a color-shifting material. However, there is no existence about the concrete structure for the cover transparency and the color tone of the underlying portion, resulting in the lack of a sufficient high-quality feel.

### SUMMARY OF THE INVENTION

It is therefore an object of the present invention to provide a two-piece colored golf ball which has good weather resistance and prevents color change, has a reassuring and psychologically calming effect on the golfer during play, and can be manufactured with an inexpensive cost.

The inventors have conducted extensive investigations aimed at achieving the above object. Consequently, as a way of satisfying the desires for a resistance to color change and a high-quality feel in a golf ball with an inexpensive manufacturing cost, the inventors have invented a two-piece golf ball which, although fluorescent, has a transparent feel and conveys a sense of quality. That is, the present invention is achieved by making the cover of the two-piece golf ball thinner, by that the quantities in which the individual pigments or dyes are added to the cover can be held to relatively small amounts, and by combining the color of the underlying core with the specific cover transparency and haze, thereby enabling a ball which also has an excellent resistance to color change and a high-quality feel to be provided.

In addition, the present invention enhances a high-quality feel by treating the pearlescent paint on the ball surface.

Accordingly, the invention provides the following colored golf balls.

[1] A colored golf ball comprising a core, a cover having a plurality of dimples formed on its surface, wherein the golf ball is two-piece structure composed of a core and a cover, the surface of the ball is coated with a coating comprising a pearlescent pigment, and the ball satisfies the following conditions:

(i) a color difference  $\Delta E^*$  between the core and the ball of at least 30;

(ii) the core has a transparency which is up to 10% in terms of total transmittance and up to 1.0% in terms of parallel transmittance;

(iii) the core has a lightness  $L^*$  value, expressed in the  $L^*a^*b^*$  color system based on JIS Z8729, of at least 82;

(iv) the ball has a lightness  $L^*$  value of at least 50;

(v) the lightness  $L^*$  value of the ball  $\leq$  the lightness  $L^*$  value of the core;

(vi) the cover has a thickness of from 0.1 to 2.1 mm;

(vii) the cover has a transparency which is at least 50% in terms of total transmittance and at least 1.0% in terms of parallel transmittance; and

(viii) the cover has a haze (H), mentioned in JIS K7105 (1981), of up to 98.

[2] The colored golf ball of [1], wherein the core has a chroma C, defined as  $(a^{*2}-b^{*2})^{1/2}$ , of at most 30.

[3] The colored golf ball of [1], wherein the amount of the pearlescent pigment in the coating is from 0.1 to 0.6 part by weight per 100 parts by weight of a base resin.

[4] The colored golf ball of [1], wherein a fluorescent whitener is included in the coating by the amount of from 0.05 to 0.5 part by weight per 100 parts by weight of a base resin.

[5] The colored golf ball of [4], wherein the weight ratio of the fluorescent whitener/the pearlescent pigment is from 0.08 to 5.0.

[6] The colored golf ball of [1], wherein the cover contains of from 0.001 to 0.4 part by weight of a pigment or dye per 100 parts by weight of base resin.

[7] The colored golf ball of [6], wherein the cover contains at least 1.0 part by weight of calcium carbonate as a diffuser for the dye per 100 parts by weight of base resin.

[8] The colored golf ball of [1], wherein the number of dimples is at most 330 and the sum of the individual dimple surface areas, defined for each dimple as the surface area of a flat plane enclosed by an edge of the dimple, is at least 80% of the spherical surface area of the ball were the ball to have no dimples thereon.

#### BRIEF DESCRIPTION OF THE DIAGRAMS

FIG. 1 is a schematic cross-sectional view of a two-piece golf ball illustrating an embodiment of the invention.

FIG. 2 is a top view of a golf ball showing dimple pattern No. 1 used in an example of the invention.

FIG. 3 is a top view of a golf ball showing dimple pattern No. 2 used in an example of the invention.

FIG. 4 is a top view of a golf ball showing dimple pattern No. 3 used in an example of the invention.

FIG. 5 is a top view of a golf ball showing dimple pattern No. 4 used in an example of the invention.

FIG. 6 is a top view of a golf ball showing dimple pattern No. 5 used in an example of the invention.

FIG. 7 is a top view of a golf ball showing dimple pattern No. 6 used in an example of the invention.

FIG. 8 is a top view of a golf ball showing dimple pattern No. 7 used in an example of the invention.

#### DETAILED DESCRIPTION OF THE INVENTION

The invention is described more fully below.

The golf ball of the present invention has a ball construction which includes a core and a cover having a plurality of dimples formed on its surface. For example, as shown in the cross-sectional view of a golf ball in FIG. 1, the inventive ball may be a two-piece golf ball G having an internal construction consisting of a core 1, a cover 2 on which a plurality of dimples D are formed. The golf ball of the present invention has the minimum performances for many golfers to be satisfied and can be manufactured with a low cost. And, the desired effects of the invention can be achieved as a result of the color tone and transparency exhibited by the core and the cover. Hence, in the present invention, the desired effects of the invention can be comprehensively achieved by satisfying the subsequently described conditions (i) to (viii).

The golf ball of the invention satisfies the following conditions:

(i) a color difference  $\Delta E^*$  between the core and the ball of at least 30;

(ii) the core has a transparency which is up to 10% in terms of total transmittance and up to 1.0% in terms of parallel transmittance;

(iii) the core has a lightness  $L^*$  value, expressed in the  $L^*a^*b^*$  color system based on JIS 28729, of at least 82;

(iv) the ball has a lightness  $L^*$  value of at least 50;  
(v) the lightness  $L^*$  value of the ball  $\leq$  the lightness  $L^*$  value of the core;

(vi) the cover has a thickness of from 0.1 to 2.1 mm,  
(vii) the cover has a transparency which is at least 50% in terms of total transmittance and at least 1.0% in terms of parallel transmittance; and

(viii) the cover has a haze (H), mentioned in JIS K7105 (1981), of up to 98.

Condition (i)

A color difference  $\Delta E^*$  between the core and the ball is at least 30. That is, the color difference between the core and the ball is large and, as subsequently described, the cover has a degree of transparency, as a result of which a color tone that shows through and imparts a sense of quality can be exhibited. Here, by determining the  $L^*$  value (lightness) and the  $a^*$  and  $b^*$  values (color coordinates) based on the  $L^*a^*b^*$  color system in JIS Z8729, the following can be calculated:

$$\Delta E^* = \{(\Delta L^*)^2 + (\Delta a^*)^2 + (\Delta b^*)^2\}^{1/2}.$$

The color difference  $\Delta E^*$  represents the linear distance between two colors in this color space.

Condition (ii)

It is essential for the core to have a degree of transparency which is up to 10% in terms of total transmittance and up to 1.0% in terms of parallel transmittance. If the core has a degree of transparency which is greater than this range, the transparency of the entire ball become larger and resulting in an inferior color tone. The core has a total transmittance of preferably at least 0%, but preferably not more than 8%, and more preferably not more than 6%. The parallel transmittance is preferably at least 0%, but preferably not more than 0.4%, and more preferably not more than 0.06%. The above-mentioned "total transmittance" and "parallel transmittance" are calculated in accordance with JIS K7105 (1981).

Condition (iii)

It is essential that, as expressed by the  $L^*a^*b^*$  method, the core have a lightness  $L^*$  value of at least 82. The  $L^*$  value is preferably at least 84, and more preferably at least 86, but preferably not more than 98, and more preferably not more than 97. In addition, the chroma C, defined as  $(a^*^2 + b^*^2)^{1/2}$  of the core, while not subject to any particular limitation, is preferably at most 30, and more preferably at most 20, further preferably at most 10. When the core is closer to white, the  $L^*$  value of the ball is larger, resulting in a luminous color. Therefore, it is preferable to use a white core.

Condition (iv)

The ball has a lightness  $L^*$  value of at least 50, preferably at least 52, and more preferably at least 54, but preferably not more than 95, and more preferably not more than 90. This is a necessary condition for preserving the visibility, brightness and high-quality feel of the ball.

Condition (v)

It is that the lightness  $L^*$  value for the ball  $\leq$  the lightness  $L^*$  value for core. The reason is that the  $L^*$  value of the core must be made larger in order to elicit a sense of transparency and brightness in the ball. The difference between the  $L^*$  value of the core and the  $L^*$  value of the ball is preferably at least 1, more preferably at least 5, and even more preferably at least 10.

Condition (vi)

The cover has a thickness which is at least 0.1 mm, preferably at least 0.2 mm, more preferably at least 0.3 mm, but not more than 2.1 mm, more preferably not more than 1.8 mm, and even more preferably not more than 1.4 mm. It is

necessary for the present invention to make the cover thin as above range in order to realize a low-cost in manufacturing the golf ball.

Condition (vii)

It is essential for the cover to have a degree of transparency which is at least 50% in terms of total transmittance and is at least 1.0% in terms of parallel transmittance. One reason is that, to confer a sense of quality, the cover as a whole must be finished so as to be a little transparent, thereby giving the ball a color tone that shows through the cover. Another reason is to bring out the brightness of the core. The total transmittance of the cover is preferably at least 52%, and more preferably at least 54%, but preferably not more than 100%.

Condition (viii)

It is essential for the cover used in the invention to have a haze (H), mentioned in JIS K7105 (1981), of up to 98. The cover as a whole must be finished so as to be transparent, thereby giving the ball a color tone that shows through the cover by suppressing the degree of haze. Haze is mentioned in JIS K7105 (1981) as a photochemical performance test method for plastic, and is calculated as follows.

$$\text{Haze}(H) = T_d/T_t \times 100(\%)$$

Here,  $T_t$  is the total light transmittance and  $T_d$  is the diffuse transmittance. The cover has a haze (H) of preferably at least 30 but not more than 98, more preferably not more than 95, and has a diffuse transmittance of preferably at least 10 but not more than 90, and more preferably at least 20 but not more than 80.

The core used in the invention may be obtained by vulcanizing a rubber composition prepared by blending a known rubber material such as 1,4-cis polybutadiene as the base resin together with a co-crosslinking agent (e.g., unsaturated carboxylic acids and metal salts thereof), an inorganic filler (e.g., zinc oxide and barium sulfate) and an organic peroxide (e.g., dicumyl peroxide and 1,1-bis(t-butylperoxy)cyclohexane). In the present invention, no particular limitation is imposed on the core diameter.

The cover material used in the invention is formed using primarily a resin material such as a thermoplastic resin or a thermoplastic elastomer. By adding suitable amounts of various pigments or dyes, the desired effects of the invention can be achieved.

Examples of pigments and dyes that may be added to the cover include, but are not limited to, light-harvesting pink dyes, solvent yellow dyes, solvent orange dyes, anthraquinone dyes, phthalocyanine dyes, fluorescent yellow pigments, fluorescent pink pigments and fluorescent orange pigments. Use may be made of known commercial products.

The amount of pigment or dye added to the cover is preferably from 0.001 to 0.4 part by weight per 100 parts by weight of the base resin. By keeping the amount of pigment or dye added within the above range, the resistance to color change of the ball as a whole can be enhanced.

It is advantageous to use a blue dye as the above-described dye included in the cover. The amount of addition in such a case is preferably not more than 0.1 part by weight per 100 parts by weight of the base resin. It is preferable for the cover surface to have a color with an  $L^*$  value of at least 50, an  $a^*$  value of from -20 to 20, and a  $b^*$  value of -20 or below. In particular, the  $L^*$  value is preferably at least 53, and more preferably at least 55, but preferably not more than 90, more preferably not more than 85, and even more preferably not more than 80. This is because, given that the color of the turf on a golf course is green in the summer and yellow in the winter, bluish balls which are positioned opposite the  $a^*$  axis

and the  $b^*$  axis from green and yellow are the easiest to find. Moreover, as is generally known, blue has a mood calming effect.

When a dye is included in the cover, it is preferable to use calcium carbonate as the diffuser for the dye. In such a case, the amount of calcium carbonate is set to preferably at least 1.0 part by weight per 100 parts by weight of the base resin. This is because calcium carbonate has a lower refractive index than titanium oxide, and thus increases the overall transparency of the cover. The amount of calcium carbonate included is preferably at least 1.3 parts by weight, and more preferably at least 1.5 parts by weight, but preferably not more than 3 parts by weight, more preferably not more than 2.8 parts by weight, and even more preferably not more than 2.6 parts by weight.

Generally, a large number of dimples are formed on the surface of a golf ball. In the present invention, the number of dimples formed on the ball surface, while not subject to any particular limitation, is preferably at least 250 but not more than 330. The dimples formed on the ball surface have a surface coverage (SR) which, while not subject to any particular limitation, is preferably at least 80%, and more preferably at least 90%, but preferably not more than 98%, and more preferably not more than 95%. By setting the number and surface coverage of the dimples within the above ranges, land areas on the surface of the ball become relatively small, which results in a better sense of transparency and thus a higher sense of quality for the ball.

The surface of the cover may be clear-coated (coated with a clear coating), in which case it is preferable for a two-part curing urethane coating to be used for clear coating. The two-part curing urethane coating is composed of a polyol component having hydroxyl groups and polyisocyanate component having isocyanate groups.

Examples of polyols that may be used include primarily urethanes, polyesters and acrylic resins, although other resins, including epoxy resins, may be used if necessary. Examples of polyisocyanates that may be used include tolylene diisocyanate (TDI), diphenylmethane-4,4'-diisocyanate (MDI), hexamethylene diisocyanate (HDI), isophorone diisocyanate (IPDI), naphthalene diisocyanate (NDI), 1,4-phenylene diisocyanate (PDI), xylylene diisocyanate (XDI) and hydrogenated xylylene diisocyanate (HXDI), either singly or in modified forms as combinations thereof. The polyisocyanate may generally be in the form of an adduct, a biuret or an isocyanurate.

The applied coat of the above coating has a thickness of preferably at least 5  $\mu\text{m}$ , and more preferably at least 10  $\mu\text{m}$ , but preferably not more than 20  $\mu\text{m}$ , and more preferably not more than 16  $\mu\text{m}$ . An applied coat that is too thin may be a factor in reducing the durability of the coating. On the other hand, if the applied coat is too thick, the rebound of the ball may decrease, shortening the carry, in addition to which separation of the core and the cover tends to arise. As a result, the durability of the ball to repeated impact may decrease.

Any known method used in the art may be employed as the coating method. For example, the ball may be perched on the tips of needles on a needle bed, and the entire ball coated with any of various types of coatings.

In the coating, various solvents and additives are suitably added to the above-described resin serving as the base, in addition to which a pearlescent pigment is included as the essential component in the present invention. When a pearlescent pigment is used, it is preferable to include from 0.05 to 0.5 part by weight of a fluorescent whitener and from 0.1 to 0.6 part by weight of the pearlescent pigment per 100 parts by weight of the base resin. Moreover, it is preferable for the

pearlescent pigment to be used in such a way that the weight ratio of the fluorescent whitener to the pearlescent pigment (fluorescent whitener/pearlescent pigment) is from 0.08 to 5.0. If the amount of pearlescent pigment included is too large, the ease of coating application may drastically decline, the ball may have a decreased rebound, and there may be a tendency for the applied coat to peel. Also, it is important to adjust the ratio of fluorescent whitener to pearlescent pigment in order to bring out the luminosity and brightness of the ball. If the amounts of the fluorescent whitener and the pearlescent pigment added are inappropriate, the ball may not have a suitable luminosity, as a result of which the desired effects of the invention may not be achieved.

Pearlescent pigments are broadly divided into metal oxide-coated micas, basic lead carbonate, bismuth oxychloride and natural pearl essence. Of these, the selection of a metal oxide-coated mica is preferred because such pigments are nontoxic and have the best chemical stability. Titanium dioxide or iron oxide is typically used as the metal oxide; by varying the coverage (thickness of the coating layer), various colors and interference effects can be achieved. The larger the particle size of these pigments, the greater the degree of luster that can be achieved. However, at a larger pigment particle size, the luster tends to subside. Hence, it is desirable to select a pigment having a suitable particle size.

Because a golf ball to which has been applied a coating that contains such a pearlescent pigment is able to reflect light at various angles, the sense of quality is increased. Moreover, because sunlight is fully reflected, the golf ball can be made easier to find.

The golf ball of the invention, which can be manufactured so as to conform with the Rules of Golf for competitive play, may be produced to a ball diameter which is not less than 42.67 mm and to a weight which is not more than 45.93 g.

With regard to the method of manufacturing the inventive golf ball, a two-piece golf ball composed of two layers may be manufactured by vulcanizing a rubber composition composed primarily of polybutadiene or the like under known vulcanization conditions to form a molded and vulcanized rubber piece (core), then successively forming a cover over the core by a known method such as injection molding. Generally, to create a large number of dimples on the surface of the ball, the dimples are formed by a large number of projections on the inside walls of the mold cavity at the same time that the material for forming the cover (outermost layer) is injection molded.

As described above, the two-piece colored golf ball of the invention is a fluorescent ball which nonetheless retains a

sense of transparency and has a high-quality feel, in addition to which it has a good weather resistance and is capable of preventing a change in color. Moreover, the colored golf ball of the invention has a reassuring and psychologically calming effect on the golfer during play, and it has a suitable look and feel. Also, since the invention is directed to a two-piece solid golf ball and the cover is made thinner, the invention can be manufactured with an inexpensive cost.

## EXAMPLES

The following examples of the invention and Comparative Examples are provided by way of illustration and not by way of limitation.

## Examples 1 to 3, Comparative Examples 1 to 7

A rubber composition having a common formulation in the examples of the invention and the comparative examples was prepared, then masticated with a kneader or a roll mill, following which cores were fabricated under specific vulcanizing conditions, which shown in Table 1. The core was then set in a mold and the cover material shown in Table 2 was injection-molded over the core, thereby giving two-piece colored golf balls according to the examples of the invention and the comparative examples. The numbers shown in the core formulation and the resin mixture formulations in Tables 1 and 2 indicate parts by weight.

TABLE 1

|  | Core Formulation                   | White core | Red core |
|--|------------------------------------|------------|----------|
|  | Polybutadiene rubber               | 100        | 100      |
|  | Zinc acrylate                      | 29         | 29       |
|  | Peroxide                           | 1.2        | 1.2      |
|  | Antioxidant                        | 0.1        | 0.1      |
|  | Zinc oxide                         | 18.4       | 18.4     |
|  | Zinc salt of pentachlorothiophenol | 0.2        | 0.2      |
|  | Red pigment                        |            | 0.08     |

The rubber was vulcanized for 15 minutes at 155° C. The above-mentioned peroxide was a mixture of 1,1-di(t-butylperoxy)cyclohexane and silica, which is produced by NOF Corporation under the trade name Perhexa C-40. The above-mentioned antioxidant is Nocrac NS-6, which is available from Ouchi Shinko Chemical Industry Co., Ltd.

TABLE 2

| Cover material |                           | a    | b     | c     | d     | e   | f  |
|----------------|---------------------------|------|-------|-------|-------|-----|----|
| Ionomer        | HIMILAN 1557 (trade name) | 75   | 75    | 75    |       |     |    |
|                | HIMILAN 1855 (trade name) | 25   | 25    | 25    |       |     |    |
|                | HIMILAN 1605 (trade name) |      |       |       | 50    | 50  | 50 |
|                | HIMILAN 1706 (trade name) |      |       |       | 50    | 50  | 50 |
|                | Magnesium stearate        | 69   | 69    | 69    |       |     |    |
| Fatty acid     | Magnesium oxide           | 0.8  | 0.8   | 0.8   |       |     |    |
|                | Titanium oxide            |      | 0.02  |       | 0.078 | 0.1 |    |
| Cation         | Calcium carbonate         | 1.5  | 1.5   | 1.3   |       |     |    |
|                | Light-harvesting dye      |      | 0.01  |       |       |     |    |
|                | Solvent yellow (dye)      | 0.09 |       | 0.035 |       |     |    |
|                | Solvent orange (dye)      |      |       | 0.004 |       |     |    |
|                | Anthraquinone (dye)       |      | 0.002 |       |       |     |    |

TABLE 2-continued

| Cover material               | a | b | c | d    | e    | f |
|------------------------------|---|---|---|------|------|---|
| Phthalocyanine (dye)         |   |   |   |      |      |   |
| Fluorescent pigment (yellow) |   |   |   | 1.56 |      |   |
| Fluorescent pigment (pink)   |   |   |   |      | 0.2  |   |
| Fluorescent pigment (orange) |   |   |   |      | 0.98 |   |

HIMILAN 1557 A zinc-neutralized ethylene-methacrylic acid copolymer available from DuPont-Mitsui Polymers Co., Ltd.

HIMILAN 1855 A zinc-neutralized ethylene-methacrylic acid-acrylic acid ester copolymer available from DuPont-Mitsui Polymers Co., Ltd.

HIMILAN 1605 A sodium-neutralized ethylene-methacrylic acid copolymer available from DuPont-Mitsui Polymers Co., Ltd.

HIMILAN 1706 A zinc-neutralized ethylene-methacrylic acid copolymer available from DuPont-Mitsui Polymers Co., Ltd.

Magnesium Stearate Available from NOF Corporation under the trade name Magnesium Stearate G.

Magnesium Oxide Magnesium oxide produced by Kyowa Chemical Industry.

Titanium Oxide Available from Ishihara Sangyo Kaisha under the trade name Tipaque R550.

TABLE 3

|                                                     | Example   |           |           | Comparative Example |       | 25 |
|-----------------------------------------------------|-----------|-----------|-----------|---------------------|-------|----|
|                                                     | 1         | 2         | 3         | 1                   | 2     |    |
| Target color                                        | yellow    | Pink      | Orange    | yellow              | pink  |    |
| Coating                                             | pearl     | pearl     | pearl     | clear               | clear |    |
| Core color                                          | white     | white     | white     | white               | white |    |
| Core diameter (mm)                                  | 40.2      | 40.2      | 40.2      | 40.2                | 40.2  |    |
| Core color L*                                       | 94.2      | 94.2      | 94.2      | 94.2                | 94.2  |    |
| a*                                                  | -1.6      | -1.6      | -1.6      | -1.6                | -1.6  |    |
| b*                                                  | -5.2      | -5.2      | -5.2      | -5.2                | -5.2  |    |
| Total transmittance                                 | 4.5       | 4.5       | 4.5       | 4.5                 | 4.5   |    |
| Haze                                                | 99.2      | 99.2      | 99.2      | 99.2                | 99.2  |    |
| Diffuse transmittance                               | 4.5       | 4.5       | 4.5       | 4.5                 | 4.5   |    |
| Parallel transmittance                              | 0.02      | 0.02      | 0.02      | 0.02                | 0.02  |    |
| (a* <sup>2</sup> + b* <sup>2</sup> ) <sup>1/2</sup> | 5.4       | 5.4       | 5.4       | 5.4                 | 5.4   |    |
| Cover formulation                                   | a         | b         | c         | a                   | b     |    |
| Cover gauge (mm)                                    | 1.25      | 1.25      | 1.25      | 1.25                | 1.25  |    |
| Total transmittance                                 | 85.8      | 54.4      | 71.2      | 85.8                | 54.4  |    |
| Haze                                                | 92.0      | 92.8      | 92.5      | 92.0                | 92.8  |    |
| Diffuse                                             | 78.9      | 48.6      | 65.8      | 78.9                | 48.6  |    |
| Parallel transmittance                              | 6.9       | 3.8       | 5.4       | 6.9                 | 3.8   |    |
| Ball color L*                                       | 93.1      | 67.3      | 83.3      | 92.8                | 66.1  |    |
| a*                                                  | -22.8     | 46.8      | 21.2      | -24.7               | 54.5  |    |
| b*                                                  | 91.5      | 6.4       | 73.8      | 98.2                | 2.4   |    |
| Color difference ΔE*                                | 99.0      | 56.6      | 82.9      | 106.0               | 63.2  |    |
| ΔE* between core and ball                           |           |           |           |                     |       |    |
| Color change resistance                             | good      | good      | good      | good                | good  |    |
| High-quality feel                                   | excellent | excellent | excellent | good                | good  |    |
| Visibility on turf                                  | excellent | excellent | excellent | good                | good  |    |

TABLE 4

|                    | Comparative Example |        |       |        |       | 60 |
|--------------------|---------------------|--------|-------|--------|-------|----|
|                    | 3                   | 4      | 5     | 6      | 7     |    |
| Target color       | orange              | yellow | pink  | orange | pink  |    |
| Coating            | clear               | pearl  | pearl | pearl  | pearl |    |
| Core color         | white               | white  | white | white  | red   |    |
| Core diameter (mm) | 40.2                | 40.2   | 40.2  | 40.2   | 37.3  |    |
| Core color L*      | 94.2                | 94.2   | 94.2  | 94.2   | 71.3  |    |
| a*                 | -1.6                | -1.6   | -1.6  | -1.6   | 38.0  |    |
| b*                 | -5.2                | -5.2   | -5.2  | -5.2   | 7.8   |    |

20

TABLE 4-continued

|                                                     | Comparative Example |       |       |      |      | 40 |
|-----------------------------------------------------|---------------------|-------|-------|------|------|----|
|                                                     | 3                   | 4     | 5     | 6    | 7    |    |
| Total transmittance                                 | 4.5                 | 4.5   | 4.5   | 4.5  | 4.6  |    |
| Haze                                                | 99.2                | 99.2  | 99.2  | 99.2 | 99.4 |    |
| Diffuse transmittance                               | 4.5                 | 4.5   | 4.5   | 4.5  | 4.6  |    |
| Parallel transmittance                              | 0.02                | 0.02  | 0.02  | 0.02 | 0.02 |    |
| (a* <sup>2</sup> + b* <sup>2</sup> ) <sup>1/2</sup> | 5.4                 | 5.4   | 5.4   | 5.4  | 38.8 |    |
| Cover formulation                                   | c                   | d     | e     | f    | b    |    |
| Cover gauge (mm)                                    | 1.25                | 1.25  | 1.25  | 1.25 | 1.25 |    |
| Total transmittance                                 | 71.2                | 48.5  | 30.6  | 44.8 | 54.4 |    |
| Haze                                                | 92.5                | 99.5  | 99.1  | 99.3 | 92.8 |    |
| Diffuse transmittance                               | 65.8                | 48.3  | 30.3  | 44.5 | 48.6 |    |
| Parallel transmittance                              | 5.4                 | 0.2   | 0.3   | 0.3  | 3.8  |    |
| Ball color L*                                       | 82.5                | 93.2  | 71.9  | 67.9 | 47.8 |    |
| a*                                                  | 24.3                | -24.4 | 57.6  | 53.5 | 49.2 |    |
| b*                                                  | 88.6                | 96.4  | -23.8 | 53.2 | 5.2  |    |
| Color difference ΔE*                                | 98.0                | 104.1 | 65.9  | 84.5 | 26.2 |    |
| between core and ball                               |                     |       |       |      |      |    |
| Color change resistance                             | good                | fair  | fair  | fair | good |    |
| High-quality feel                                   | good                | fair  | fair  | fair | NG   |    |
| Visibility on turf                                  | good                | good  | good  | good | NG   |    |

The appearance-related properties of the core, cover and golf ball obtained in each of the examples of the invention and the comparative examples were rated according to the following criteria. The results are shown in Tables 3 and 4.

#### Total Transmittance and Parallel Transmittance

Measurement was carried out using a light transmittance measuring instrument (Turbidimeter NDH5000W, manufactured by Nippon Denshoku Industries Co., Ltd.), and the total transmittance and parallel transmittance were determined based on JIS K7105. Higher values for total transmittance and parallel transmittance indicate that light passes through more easily; i.e., that the degree of transparency is higher. Conversely, lower values indicate that light passes through with greater difficulty; i.e., that the degree of transparency is smaller.

Lower values for haze and diffuse transmittance indicate lower levels of haze and light diffusion, signifying better transparency.

#### Color Difference ΔE\*

Measurement was carried out using a color difference meter (model SC-P, manufactured by Suga Test Instruments Co., Ltd.), and the color difference ΔE\* was determined based on the L\*a\*b\* color system in JIS Z8729. A larger value indicates a larger color difference, and a smaller value indicates a smaller color difference.

## 11

## Color Change Resistance

The ball was irradiated for 24 hours with a mercury vapor lamp. The degree of color change upon exposure to ultraviolet light was observed, and rated as follows.

Good: Substantially no change in color

Fair: Slight change in color

NG: Large change in color

## High-Quality Feel

Sensory evaluations based on the following criteria were carried out by ten skilled golfers.

|            |                                                                          |
|------------|--------------------------------------------------------------------------|
| Excellent: | Eight or more of the 10 golfers thought the ball had a high-quality feel |
| Good:      | Five to seven of the 10 golfers thought the ball had a high-quality feel |
| Fair:      | Three or four of the 10 golfers thought the ball had a high-quality feel |
| NG:        | Two or fewer of the 10 golfers thought the ball had a high-quality feel  |

## Visibility on Turf

Sensory evaluations based on the following criteria were carried out by ten skilled golfers.

|            |                                                                          |
|------------|--------------------------------------------------------------------------|
| Excellent: | Eight or more of the 10 golfers thought the ball was easy to see on turf |
| Good:      | Five to seven of the 10 golfers thought the ball was easy to see on turf |
| Fair:      | Three or four of the 10 golfers thought the ball was easy to see on turf |
| NG:        | Two or fewer of the 10 golfers thought the ball was easy to see on turf  |

From the results in Tables 3 and 4, the respective comparative examples were inferior in the following ways to the examples according to the present invention.

In each of Comparative Examples 1, 2 and 3, since not clear coating but pearl coating was treated on the respective ball surface, the ball lacked a high-quality feel.

In Comparative Examples 4, 5 and 6, since the transparency of the cover was low, the color change resistance and the high-quality feel were poor. In addition, the haze value of the cover is too large, the transparency fell of the ball was poor and the ball lacked a high-quality feel.

In Comparative Example 7, since the color difference  $\Delta E^*$  between the core and the ball is less than 30, the ball lacked visibility on turf and a high-quality feel.

Various types of dimple patterns were placed on the ball construction in Example 1, and the sense of cover transparency was examined. These dimple patterns Nos. 1 to 7 are shown in Table 5 below and in accompanying FIGS. 2 to 8. Each dimple pattern was formed on the cover surface at the same time that the cover resin material was injection molded.

TABLE 5

|                                                                       | Dimple pattern |        |        |        |        |        |        |
|-----------------------------------------------------------------------|----------------|--------|--------|--------|--------|--------|--------|
|                                                                       | No. 1          | No. 2  | No. 3  | No. 4  | No. 5  | No. 6  | No. 7  |
| Arrangement in pattern of dimples                                     | FIG. 2         | FIG. 3 | FIG. 4 | FIG. 5 | FIG. 6 | FIG. 7 | FIG. 8 |
| Total number of dimples                                               | 326            | 326    | 344    | 330    | 368    | 306    | 432    |
| Ratio of dimple areas (%)<br>(ratio of surface other than lands (SR)) | 90             | 81.3   | 82.1   | 80.5   | 78.2   | 77.8   | 75.2   |

## 12

## Ratio of Dimple Areas (SR)

This ratio is the sum of the individual dimple surface areas, defined for each dimple as the surface area of the flat plane enclosed by the dimple edge, as a percentage of the spherical surface area of the ball were the ball to have no dimples thereon.

The sense of cover transparency was evaluated. When sensory evaluations were carried out by ten skilled golfers, eight or more of the golfers rated covers bearing the dimple pattern in FIG. 2 as having a sense of transparency; from five to seven of the golfers rated covers bearing the dimple patterns in FIGS. 3, 4 and 5 as having a sense of transparency; three or four of the golfers rated covers bearing the dimple pattern in FIG. 6 as having a sense of transparency; and two or fewer golfers rated covers bearing the dimple patterns in FIGS. 7 and 8 as having a sense of transparency.

## The invention claimed is:

1. A colored golf ball comprising a core, a cover having a plurality of dimples formed on its surface, wherein the golf ball is two-piece structure composed of a core and a cover, the surface of the ball is coated with a coating comprising a pearlescent pigment, and the ball satisfies the following conditions:
  - (i) a color difference  $\Delta E^*$  between the core and the ball of at least 30;
  - (ii) the core has a transparency which is up to 10% in terms of total transmittance and up to 1.0% in terms of parallel transmittance;
  - (iii) the core has a lightness  $L^*$  value, expressed in the  $L^*a^*b^*$  color system based on JIS Z8729, of at least 82;
  - (iv) the ball has a lightness  $L^*$  value of at least 50;
  - (v) the lightness  $L^*$  value of the ball  $\leq$  the lightness  $L^*$  value of the core;
  - (vi) the cover has a thickness of from 0.1 to 2.1 mm,
  - (vii) the cover has a transparency which is at least 50% in terms of total transmittance and at least 1.0% in terms of parallel transmittance; and
  - (viii) the cover has a haze (H), mentioned in JIS K7105 (1981), of up to 98.
2. The colored golf ball of claim 1, wherein the core has a chroma C, defined as  $(a^{*2}+b^{*2})^{1/2}$ , of at most 30.
3. The colored golf ball of claim 1, wherein the amount of the pearlescent pigment in the coating is from 0.1 to 0.6 part by weight per 100 parts by weight of a base resin.
4. The colored golf ball of claim 1, wherein a fluorescent whitener is included in the coating by the amount of from 0.05 to 0.5 part by weight per 100 parts by weight of a base resin.
5. The colored golf ball of claim 4, wherein the weight ratio of the fluorescent whitener/the pearlescent pigment is from 0.08 to 5.0.
6. The colored golf ball of claim 1, wherein the cover contains of from 0.001 to 0.4 part by weight of a pigment or dye per 100 parts by weight of base resin.

7. The colored golf ball of claim **6**, wherein the cover contains at least 1.0 part by weight of calcium carbonate as a diffuser for the dye per 100 parts by weight of base resin.

**8.** The colored golf ball of claim **1**, wherein the number of dimples is at most 330 and the sum of the individual dimple surface areas, defined for each dimple as the surface area of a flat plane enclosed by an edge of the dimple, is at least 80% of the spherical surface area of the ball were the ball to have no dimples thereon. 5

\* \* \* \* \*

10